# EUROPEAN PATENT SPECIFICATION

(11) **EP 2 447 398 B1**
(45) Date of publication and mention of the grant of the patent: **05.06.2013**
(21) Application number: 10189550.6
(22) Date of filing: 01.11.2010
(51) Int. Cl.: D01G 13/00

(54) **Method for mixing short staple and down cluster by a dry processing**
Verfahren zum Mischen von Kurzstapeln und nach unten gerichteten Clustern mittels Trockenverarbeitung
Procédé de mélange d'une agrafe courte et d'un groupe descendant par un traitement à sec

(43) Date of publication of application: 02.05.2012
(73) Proprietor: Kwong Lung Enterprise Co., Ltd., Taipei (TW)
(72) Inventor: Wen, Hsiu-Jung, Taipei (TW)
(74) Representative: Viering, Jentschura & Partner

(56) References cited:
- CN-Y- 2 534 200
- JP-A- 10 219 526
- JP-A- 10 331 061

## Description

### BACKGROUND OF THE INVENTION

### 1. Field of the Invention

The present invention relates to a method for mixing short staple and down cluster by a dry processing, in particular to a method that employs an air tool to blow a short staple cluster over, thereby allowing the short staple cluster to be further mixed with the down cluster.

### 2. Description of the Related Art

Since feathers (down feather) are lightly excellent in warmth retaining property, they are used abundantly at a down wear, a down quilt, a sleeping bag, etc. Tucking in afore products allows warmth to be retained around users. Preferably, the light feature of the down product provides users with a flexible motion.

However, extracted from waterfowls, such as a goose and a duck, the down usually contains high water repellence. Herein, in view of the advanced water repellence, the down has to be dissolved in a hot water bath with drugs for stirring, so that a functional processing treatment could be carried out. However, the treatment is actually inconvenient because of the minute and complicated preparation. Even the functional processing treatment is launched, the processed down adversely has a poor property of washing resistance. Moreover, the treatment cost is high, which results in the lack of practicability. A Japanese Patent No. 3383855 stirs staple fibers and feathers that have the wettability after washing in a mixing process bath containing a surfactant system softening agent. The staple fibers are entwined with the barbule. Herein, the disclosed processing treatment needs an environment of high humidity for mixing the feather and the staple fibers. Obviously, such processing treatment simply takes time and the applied material is easily worn out. Thus, the limited operating environment and the long processing time are both unbenefited to the speedy productivity, which causes the applicant' s endeavor to solve the disadvantages.

CN-2,534,2004 discloses a further prior art.

### SUMMARY OF THE INVENTION

Accordingly, the applicant of the present invention made an effort to solve the disadvantages existing in the conventional method with a novel technique, so that an improved product could be expected for an advanced development in the industry.

A method for mixing short staple and down cluster by a dry processing is provided according to claim 1.

A windmill motor is disposed at one side of the stirring tank; said windmill motor is communicated with an air tube that includes two air holes respectively defined at both sides of the stirring tank; a filter is installed on the air hole, and an entrance is disposed in the blending trough; the mixture of the strands of short staple with the down cluster is sucked into the stirring tank via the entrance while turning on the windmill motor in step (b).

A channel disposed at the other side of the stirring tank for being corresponding to the windmill motor is communicated with the gathering room.

The gathering room includes two accommodating rooms respectively communicated with the channel; a blocking member is disposed at a convergence of the channel and the accommodating rooms.

A proportion of the strands of short staple mixed with the down cluster is 1% to 30%; a preferable proportion of said mixture is 5% to 20%.

The present invention contributes to the following advantages:
By means of abovementioned steps, the stirring time and the stirring procedure in the stirring tank are shortened about within 20 minutes. Thus, the speedy productivity is achieved by the shortened stirring procedure.

Further, in time of mixing, no chemical drug is needed, and the mixture of the short staple and the down also does not have to be soaked in any liquid. Accordingly, troubles correlated with the drainage, the heating facility, and the resulted pollution are all prevented for saving cost.

In addition, the proportion of the short staple to the down cluster can be adjusted in accordance with the practical property of the product to be made. For example, if the effect of retaining warmth is to be enhanced, the proportion of the short staple will be raised. On the other hand, the proportion of the short staple could be alternatively decreased for saving cost.

Following embodiments and correlated figures are believed to show a clear performance of the present invention.

### BRIEF DESCRIPTION OF THE DRAWINGS

Fig. **1** is a schematic view showing a blending trough of the present invention;
Fig. **2** is a flowchart showing the processing procedure of the present
   invention;
Fig. **3** is a schematic view showing the short staple cluster of the present invention;
Fig. **4** is a schematic view showing strands of short staple formed by the scattered short staple cluster;
Fig. **5** is a schematic view showing a down cluster of the present invention;
Fig. **6** is a schematic view showing a mixture of the short staple and the down cluster; and
Fig. **7** is an experimental statistic of the present invention.

### DETAILED DESCRIPTION OF THE PREFERRED EMBODIMENTS

Figs. **1** and **2** show a method for mixing short staple and down cluster by a dry processing comprising steps of:
(a) turning on an air tool **2** in a blending trough **1** for creating an air current and blowing the air current over a short staple cluster **F** disposed in the blending trough **1** (as shown in Fig. **3**), so that the short staple cluster **F** subjected to blows of the air current is separated into strands **F1** of short staple (as shown in Fig. **4**) (**901**) ;
(b) mixing the strands **F1** of short staple with a down cluster **D** (as shown in Fig. **5**); a mixture of the strands of short staple and the down cluster (as shown in Fig. **6**) being conveyed to a stirring tank **3** disposed at a bottom of the blending trough **1** (**902**);
(c) repeating step (a) to step (b) until the short staple cluster **F** is used up (**903**);
(d) placing the redundant down cluster **D** into the stirring tank **3** and turning on stirring blades **4** disposed in the stirring tank **3** (**904**); and
(e) taking the mixture of the strands **F1** of short staple and the down cluster **D** into a gathering room **5** disposed in the blending trough **1** after a stirring process is completed (**905**).

A windmill motor **6** is disposed at one side of the stirring tank **3.** The windmill motor **6** is communicated with an air tube **61** that includes two air holes **62** respectively defined at both sides of the stirring tank **3.** A filter **63** is further installed on the air hole **62,** and an entrance **10** is disposed in the blending trough **1.** Thereby, the mixture of the strands **F1** of short staple and the down cluster **D** is sucked into the stirring tank **3** via the entrance **10** while turning on the windmill motor **6** in step (b).

Further, a channel **7** disposed at the other side of the stirring tank **3** for being corresponding to the windmill motor **6** is further communicated with the gathering room **5.**

Moreover, the gathering room **5** includes two accommodating rooms **50, 51** respectively communicated with the channel **7.** A blocking member **52** is disposed at a convergence of the channel **7** and the accommodating room **50.**

According to the steps and the correlated figures above, the present invention is operated within the blending trough **1** that includes one air tool **2,** one stirring tank **3,** one set of stirring blades **4,** one gathering room **5,** one windmill motor **6,** and one channel **7.**

The stirring tank **3** is disposed at the bottom of the bending trough **1.** The entrance **10** is disposed between the stirring tank **3** and the blending trough **1.** The entrance **10,** the stirring tank **3,** and the blending trough **1** are intercommunicated with each other. The windmill motor **6** is disposed at one side of the stirring tank **3** and communicated with the air tube **61.** The air tube **61** includes two air holes **62** that are respectively disposed at the side of the stirring tank **3.** The filter **63** is disposed on the air hole **62.** The flowing air current is created by the air tube **61.** Disposed on the other side of the windmill motor **6,** the channel **7** is communicated with the gathering room **5.**

Two accommodating rooms **50, 51** included by the gathering room **5** are respectively communicated with the channel **7.** The blocking member **52** is disposed at the convergence of the channel **7** and the accommodating room **50.**

The set of the stirring blades **4** includes a stirring motor **41** and a blade unit **42.** The stirring motor **41** is disposed out of the stirring tank **3.** The blade unit **42** is disposed in the stirring tank. Preferably, the stirring motor **41** and the blade unit **42** are connected with each other.

A controller **8** disposed in the blending trough **1** further includes a feeding switch **81,** a stirring switch **82,** and an extruding switch **83.** The feeding switch **81** and the extruding switch **83** are electrically connected to the windmill motor **6.** The stirring switch **82** is electrically connected to the stirring motor **41.**

In operation, the short staple cluster **F** and the down cluster **D** are placed in the blending trough **1.** Thereby, the air tool **2** creates an air current. Thence, blowing over via the air current, the short staple cluster **F** is scattered into strands **F1** of short staple. The strands **F1** of short staple are mixed with the down cluster **D**. Accordingly, while the feeding switch **81** is turned on to motivate the windmill motor **6** for the air current to travel through the air tube **61** from the air hole **62,** a mixture of the strands **F1** of short staple and the down cluster is sucked in the stirring tank **3** via the entrance **10.** Herein, the filter **63** prevents the strands **F1** of short staple and the down cluster **D** from being sucked into the windmill motor **6.** Aforementioned operation is repeatedly conducted until the short staple cluster **F** is used up.

Afterward, the redundant down fluster **D** is placed in the stirring tank **3** via the entrance **10.** Thence, the stirring switch **82** is turned on for motivating the stirring motor **41.** Thereby, the blade unit **42** is rotated for launching the stirring.

Certain operating time of the stirring has to be properly adopted. Namely, the rotation of the blade unit **42** has to be suspended for 2 minutes per 5-minute-operation. The procedure has to be conducted for three rounds. Accordingly, the total stirring time will be 15 minutes, and the total suspension will be 4 minutes. Such procedure contributes to the even mixture.

The extruding switch **83** is turned on after the completion of the stirring. Turning on the extruding switch **83** allows the windmill motor **6** to fan. Whereby, the mixture of the strands **F1** of short staple and the down cluster **D** in the stirring tank **3** enters into the gathering room **5** via the channel **7.** Preferably, the rotating blade unit further provides the mixture of the strands **F1** of short staple and the down cluster **D** with an additional push for achieving a smooth traveling into the channel, so that a convenient gathering is resulted.

Two accommodating rooms **50, 51** included by the gathering room **5** are respectively connected to the channel **7.** Both the strands **F1** of short staple and the down cluster **D** are gathered for entering the accommodating rooms **50, 51.** The blocking member **52** (or a valve switch) is further disposed at the exit of the channel **7** with respect to the accommodating room **50.** By means of the blocking member **52,** a blockage between the accommodating rooms **50, 51** and the channel **7** is formed therebetween. Thereby, the mixture of the strands **F1** of short staple and the down cluster **D** would selectively enter the accommodating rooms **50, 51.** Succeedingly, a weaving bag **P** is disposed on the convergence among the exit of the channel **7** and the accommodating rooms **50, 51** for collecting the mixture of the strands **F1** of short staple and the down cluster.

The present invention conduces to a speedy mixture and avoids the pollutant generated in the conventional wet processing, which contributes to an inventive step.

In fact, the aim of mixing the strands **F1** of short staple and the down cluster **D** is to achieve a mixture that retains warmth since the strands **F1** of short staple are featured by retaining the absorbed warmth. Herein, the proportion for mixing the strands **F1** of short staple with the down cluster **D** will be discussed later in the specification. It should be noted that a proportion of the strands **F1** of short staple mixed with the down cluster **D** is 1% to 30%. Preferably, a proportion of the strands **F1** of short staple mixed with the down cluster is 5% to 20%.

An experimentation for observing a relationship between the effect of retaining warmth and the proportion of the strands of short staple **F1** in the mixture is conducted by the following means: A halogen lamp of 500W is set away from a sample by 100 centimeters for 10 minutes. Thence, an infrared thermal imager measures the surface temperature of the sample. Accordingly, a comparison between a before-temperature and an after-temperature of the surface of the sample will be conducive to a conclusion as follows.

Referring to Fig. **7****,** an obvious warmth retaining effect is achieved while the proportion of the strands **F1** of short staple is set from 1% to 20%. Moreover, when the weight proportion of the strands **F1** of short staple is assumed from 1% to 20%, the mixture of the strands **F1** of short staple and the down cluster **D** has a better warmth retaining effect than that of the cluster **D** without the strands **F1** of short staple.

The following Forms 1 to 3 present three different tests on the temperature that proves the superior warmth retaining effect while adding the strands **F1** of short staple (increased temperature as follows is indicated to the surface increased temperature of the sample; compared temperature as follows is indicated to the comparison of the increased temperature of the sample added with the strands F1 of short staple to the increased temperature of the sample without the strands F1 of short staple):

**FORM 1**

| | NO SHORT STAPLE | 1% | 5% | 10% | 15% | 20% |
|---|---|---|---|---|---|---|
| INCREASED TEMPERATURE | +5.57□ | +5.95°C | +7.17□ | +9.66□ | +9.28□ | +8.55□ |
| COMPARED TEMPERATURE | +0□ | +0.38□ | +1.60□ | +4.09□ | +3.71□ | +2.98□ |

**FORM 2**

| | NO SHORT STAPLE | 1% | 5% | 10% | 15% | 20% |
|---|---|---|---|---|---|---|
| INCREASED TEMPERATURE | +6.04°C | 6.45°C | +7.98°C | +8.89°C | +8.3°C | +8.06°C |
| COMPARED TEMPERATURE | +0°C | +0.41°C | +1.94°C | +2.85°C | +2.26°C | +2.02°C |

**FORM 3**

| | NO SHORT STAPLE | 1% | 5% | 10% | 15% | 20% |
|---|---|---|---|---|---|---|
| INCREASED TEMPERATURE | +7.4°C | +8.24 | +9.61°C | +10.55 °C | +9.79°C | +9.72°C |
| COMPARED TEMPERATURE | +0°C | +0.84 | 2.21°C | +3.15°C | +2.39°C | +2.32°C |

## Claims

1. A method for mixing short staple and down cluster by a dry processing comprising steps of:
(a) turning on an air tool (2) in a blending trough (1) for creating an air current therein and blowing said air current over a short staple cluster (F) disposed in said blending trough (1), so that said short staple cluster (F) subjected to blows of said air current is separated into strands (F1) of short staple;
(b) mixing said strands (F1) of short staple with a down cluster (D); a mixture of said strands (F1) of short staple and said down cluster (D) being conveyed to a stirring tank (3) disposed at a bottom of said blending trough (1);
(c) repeating step (a) to step (b) until said short staple cluster (F) is used up;
(d) placing the redundant down cluster (D) into said stirring tank (3) and turning on stirring blades (4) disposed in said stirring tank (3); and
(e) taking said mixture of said strands (F1) of short staple and said down cluster (D) into a gathering room (5) disposed in said blending trough (1) after a stirring process is completed, wherein
one windmill motor (6) is disposed at one side of said stirring tank (3); said windmill motor (6) is communicated with an air tube (61) that includes two air holes (62) respectively defined at both sides of said stirring tank (3); a filter (63) is installed on said air hole (62), and an entrance (10) is disposed in said blending trough (1) ; while a feeding switch (81) is turned on, said mixture of said strands (F1) of short staple with said down cluster (D) is sucked into said stirring tank (3) via said entrance (10) while turning on said windmill motor (6) in step (b), and turning on an extruding switch (83) allows said windmill motor (6) to fan in step (e), whereby said mixture of the strands (F1) of short staple and the down cluster (D) in the stirring tank (3) enters into the gathering room (5) via a channel (7).

2. The method as claimed in claim 1, wherein, the channel (7) disposed at the other side of said stirring tank (3) for being corresponding to the windmill motor (6) is communicated with said gathering room (5).

3. The method as claimed in claim 2, wherein, said gathering room (5) includes two accommodating rooms (50,51) respectively communicated with said channel (7); a blocking member (52) is disposed at a convergence of said channel (7) and said accommodating rooms (50,51).

4. The method as claimed in claim 1, wherein, a proportion of said strands (F1) of short staple mixed with said down cluster (D) is 1% to 30%.

5. The method as claimed in claim 4, a proportion of said strands (F1) of short staple mixed with said down cluster (D) is 5% to 20%.

## Patentansprüche

1. Ein Verfahren zum Mischen von Kurzfaser und einem Daunenhaufen durch eine Trockenverarbeitung, aufweisend die Schritte des:
(a) Anschalten eines Luftwerkzeugs (2) in einem Mischbottich (1) zum Erzeugen eines Luftstroms darin und zum Blasen des Luftstroms über einen Kurzfaserhaufen (F), welcher in dem Mischbottich (1) angeordnet ist, so dass der Kurzfaserhaufen (F), welcher Luftstößen des Luftstroms unterliegt, in Stränge (F1) der Kurzfaser aufgeteilt ist,
(b) Vermischen der Stränge (F1) der Kurzfaser mit einem Daunenhaufen (D), wobei eine Mischung aus den Strängen (F1) der Kurzfaser und dem Daunenhaufen (D) zu einem Rührbehälter (3) befördert wird, welcher an einem Unterteil des Mischbottichs (1) angeordnet ist,
(c) wiederholen von Schritt (a) bis Schritt (b) bis der Kurzfaserhaufen (F) aufgebraucht ist,
(d) Platzieren des nicht verbrauchten Daunenhaufens (D) in dem Rührbehälter (3) und Anschalten von Rührblättern (4), welche in dem Rührbehälter (3) angeordnet sind, und
(e) Bringen der Mischung aus den Strängen (F1) der Kurzfaser und dem Daunenhaufen (D) in einen Sammelraum (5), welcher in dem Mischbottich (1) angeordnet ist, nachdem ein Rührvorgang abgeschlossen ist, wobei
ein Luftschraubenmotor (6) an einer Seite des Rührbehälters (3) angeordnet ist, wobei der Luftschraubenmotor (6) mit einem Luftrohr (61) in Verbindung steht, welches zwei Luftlöcher (62) aufweist, die jeweilig an einer der beiden Seiten des Rührbehälters (3) definiert sind, wobei ein Filter (63) an dem Luftloch (62) installiert ist, und wobei ein Einlass (10) in dem Mischbottich (1) angeordnet ist, wobei beim Eingeschaltet sein eines Zuführungsschalter (81) die Mischung aus den Strängen (F1) der Kurzfaser mit dem Daunenhaufen (D) in den Rührbehälter (3) durch den Einlass (10) eingesaugt wird, wobei der Luftschraubenmotor (6) in Schritt (b) eingeschaltet ist, und wobei Einschalten eines Ausstoßschalters (83) es dem Luftschraubenmotor (6) erlaubt, in Schritt (e) zu blasen, wodurch die Mischung aus den Strängen (F1) der Kurzfaser und dem Daunenhaufen (D) in dem Rührbehälter (3) durch einen Kanal (7) in den Sammelraum (5) eintritt.

2. Das Verfahren gemäß Anspruch 1, wobei der Kanal (7), welcher an der anderen Seite des Rührbehälters (3) angeordnet ist, um korrespondierend zu dem Luftschraubenmotor (6) zu sein, mit dem Sammelraum (5) in Verbindung steht.

3. Das Verfahren gemäß Anspruch 2, wobei der Sammelraum (5) zwei Aufnahmeräume (50,51) aufweist, welche jeweils mit dem Kanal (7) in Verbindung stehen, wobei ein Blockierelement (52) an einer Zusammenführung des Kanals (7) und der Aufnahmeräume (50,51) angeordnet ist.

4. Das Verfahren gemäß Anspruch 1, wobei ein Anteil der Stränge (F1) der Kurzfaser, welche mit dem Daunenhaufen (D) vermischt ist, 1% bis 30% beträgt.

5. Das Verfahren gemäß Anspruch 4, wobei ein Anteil der Stränge (F1) der Kurzfaser, welche mit dem Daunenhaufen (D) vermischt ist, 5% bis 20% beträgt

## Revendications

1. Procédé destiné à mélanger des fibres courtes et une touffe de duvet à l'aide d'un traitement à sec comprenant les étapes consistant à :
(a) mettre en marche un outil pneumatique (2) dans un bac de mélange (1) pour créer un courant d'air à l'intérieur et souffler ledit courant d'air sur une touffe de fibres courtes (F) disposée dans ledit bac de mélange (1), de telle sorte que ladite touffe de fibres courtes (F) soumise aux souffles dudit courant d'air soit séparée en brins (F1) de fibres courtes ;
(b) mélanger lesdits brins (F1) de fibres courtes avec une touffe de duvet (D) ; un mélange desdits brins (F1) de fibres courtes et de ladite touffe de duvet (D) étant acheminé vers un réservoir d'agitation (3) disposé au niveau du fond dudit bac de mélange (1) ;
(c) répéter l'étape (a) et l'étape (b) jusqu'à ce que ladite touffe de fibres courtes (F) soit épuisée ;
(d) placer la touffe de duvet inutilisée (D) dans ledit réservoir d'agitation (3) et mettre en marche les pales d'agitation (4) disposées dans ledit réservoir d'agitation (3) ; et
(e) placer ledit mélange desdits brins (F1) de fibres courtes et de ladite touffe de duvet (D) dans une chambre d'accumulation (5) disposée dans ledit bac de mélange (1) à la fin d'un processus d'agitation, dans lequel :
un moteur de soufflante (6) est disposé au niveau d'un côté dudit réservoir d'agitation (3) ; ledit moteur de soufflante (6) est en communication avec un conduit d'air (61) qui comprend deux trous d'air (62) définis respectivement au niveau des deux côtés dudit réservoir d'agitation (3) ; un filtre (63) est installé sur ledit trou d'air (62), et une entrée (10) est disposée dans ledit bac de mélange (1) ; tandis qu'un commutateur d'alimentation (81) est mis en marche, ledit mélange desdits brins (F1) de fibres courtes et de ladite touffe de duvet (D) est aspiré dans ledit réservoir d'agitation (3) via ladite entrée (10) en mettant en marche ledit moteur de soufflante (6) dans l'étape (b), et la mise en marche d'un commutateur d'extrusion (83) permet audit moteur de soufflante (6) de souffler dans l'étape (e), grâce à quoi ledit mélange de brins (F1) de fibres courtes et de la touffe de duvet (D) dans le réservoir d'agitation (3) pénètre dans la chambre d'accumulation (5) via un canal (7).

2. Procédé selon la revendication 1, dans lequel le canal (7) disposé au niveau de l'autre côté dudit réservoir d'agitation (3) pour correspondre au moteur de soufflante (6), communique avec ladite chambre d'accumulation (5).

3. Procédé selon la revendication 2, dans lequel ladite chambre d'accumulation (5) comprend deux chambres de réception (50, 51) qui communiquent respectivement avec ledit canal (7) ; un élément de blocage (52) est disposé au niveau d'une convergence dudit canal (7) et desdites chambres de réception (50, 51).

4. Procédé selon la revendication 1, dans lequel une proportion desdits brins (F1) de fibres courtes mélangés à ladite touffe de duvet (D), est comprise entre 1 % et 30 %.

5. Procédé selon la revendication 4, dans lequel une proportion desdits brins (F1) de fibres courtes mélangés à ladite touffe de duvet (D), est comprise entre 5 % et 20 %.
